

D. J. SIMPSON,

PROCESS OF STEEL TREATMENT.

APPLICATION FILED APR. 5, 1915. RENEWED DEC. 29, 1919.

1,351,494.

Patented Aug. 31, 1920.

Fig. 1.



Fig. 3.



David J. Simpson Inventor

Witnesses  
A. S. Anstey  
M. J. Campbell

28-14  
D. S. Anstey

Attorney



Fig. 4.



# UNITED STATES PATENT OFFICE.

DAVID J. SIMPSON, OF CHICAGO, ILLINOIS, ASSIGNOR TO NOAH STEINER AMSTUTZ,  
OF VALPARAISO, INDIANA.

## PROCESS OF STEEL TREATMENT.

1,351,494.

Specification of Letters Patent. Patented Aug. 31, 1920.

Application filed April 5, 1915, Serial No. 19,310. Renewed December 29, 1919. Serial No. 348,049.

*To all whom it may concern:*

Be it known that I, DAVID J. SIMPSON, citizen of the United States, residing at Chicago, in the county of Cook and State of Illinois, have invented certain new and useful Improvements in Processes of Steel Treatment, of which the following is a specification.

My invention relates to improvements in the process of steel treatment and it consists more especially of the steps pointed out in the annexed claims.

The purpose of my invention is to provide a method of steel treatment that will uniformly secure a more homogeneous characteristic of steel products than has hitherto been attainable; to secure such a relation between the particles of which the steel is composed as to insure a high elastic limit and tensile strength, with large reduction of area, and great elongation before fracture; that will at the same time have a high degree of hardness without sacrificing toughness; that may be carried into practice without complicated and expensive devices; that is simple in the sequence of its steps; positive in results; inexpensive to operate; and economically produces products of the highest quality.

With this process a uniformity of product is secured throughout a continuous output that has not been reached heretofore. In practice a large output of locomotive axles covering many months was found to meet the most exacting physical tests of the purchasers without coming short on a single specification, whereas the lack of uniformity in quantity output when quenching, etc., is resorted to is in marked contrast to the exceptional results attained by this process.

With these and other ends in view I illustrate in the accompanying drawings such instances of adaptation as will disclose the broad features without specifically limiting myself.

Figure 1— shows a diagrammatic relation of various means, among others, that may be used in carrying out such a process.

Fig. 2— shows a controlled air chamber. Fig. 3— shows a top plan view of an arrangement of dampers.

Fig. 4— shows a side elevation of Fig. 3.

In carrying my process into practice the billets are heated in any well known manner preparatory to being hammered into the de-

sired shape. After this the axles are placed onto any suitable form of supports shown at 1 of Fig. 1 where they are allowed to cool to atmospheric temperature. From here they are usually rolled by hand into the left end 60 of furnace A onto bars of any desired cross section, not shown, in order to allow a free circulation of the heat around the axles. This provision is an obvious one and is found in common practice. In this furnace 65 the axles are first heated very gradually up to the low critical point which varies throughout a range of about 150 degrees F. between 1390 and 1240 inversely to a change in carbon content. From about .30 to .35% 70 for the lowest percentage of carbon the higher temperature is required and for the higher carbons .60 to .65% a lower temperature from 1240 to 1270 suffices. An intermediate relation is 1310 to 1340° F. for .45 to 75 .50% carbon. Other percentages of carbon bear an inverse relation to the temperature change which throughout the whole range is found to practically follow a straight line curve. During this slow rise of heat the 80 molecular relation is readjusted so as to form a new structure. After the required temperature has been reached for a given carbon composition it is held uniform for a period of about one-third to one-half hour so as to 85 avoid a too sudden rearrangement of the particles. This rest period is vital to the success of the process and must be carefully watched, otherwise only unsatisfactory results will be secured.

The time required to reach these temperatures varies approximately with the sizes of axles to be treated, ranging from about three hours for five inch diameters to six hours for eleven to twelve inch diameters. Cold steel 95 should not be subjected to the extreme stresses which will inevitably be set up if charged into furnaces having a higher temperature than 850 to 900 degrees F. Excessive initial temperatures do not give time for 100 a gradual rearrangement of the particles to produce homogeneous results.

A second heating follows the rest period in order to bring the axles up to the high critical point which ranges from 1420 to 1440 degrees F. for .65% carbon; 1480 to 1500 for .50% carbon and 1560 to 1580 degrees F. for .30% carbon percentages. These temperature changes also follow a straight line curve. To reach these temperatures for five 110

inch sections requires about one hour and for the larger diameters approximately three hours. By the time the second heating is completed the buggy 5 can be moved near the furnace A between it and the treatment chamber B ready to enter the furnace.

The axles are placed side by side in the furnace with sufficient space between them to allow the heat to circulate. It is wide enough to form a vacant space adjacent each end of the axles into which two removable rails shown in dotted lines of Fig. 1 are quickly placed by a hoist as soon as the furnace doors are opened. These rails connect with the buggy tracks at the other end of the furnace and they serve to support the buggy as it is rapidly moved into the furnace with its main structure "straddling" the axles. The heated axles are raised by the buggy and taken to the treatment chamber where they are lowered onto isolated supports and the buggy is removed empty from the far end of the chamber traversing the transfer tracks which are placed along each side of the chamber.

A hood is lowered over the deposited axles so that its edges drop into a water seal at the bottom of the chamber. The rapid cooling is effected by first admitting air under pressure or dry steam at about 350 degrees F. into the top of the hood and withdrawing it through separately controlled exit chambers to a common outlet. When the treatment is completed the hood is raised and the buggy is again moved into position to lift the axles and transport them to any storage space beyond the chamber.

If after the first heat is completed there should be a doubt as to the ultimate quality the axles can be cooled to about 600 degrees F. and returned to the furnace for a draw back treatment which for .30% carbons is about 900 degrees F.; for .50% carbon 1150 degrees F. and for .65% carbon 1260 degrees F., other carbon contents being proportional. These draw back temperatures are to be held from one to two hours.

The furnace A may be charged by hand or otherwise from the stock rack 1. Its heat distribution may be controlled by dampers whose hand levers 2 are accessible outside of the wall. Doors 3 and 4 are raised and lowered in any suitable manner. They have inspection windows and pyrometer openings. When the heating has progressed sufficiently the doors are opened and buggy 5 is rapidly moved into it so as to leave motor 6 on the outside. Suitable side bars with "toe" flanges engage the material being treated, in this instance axles, and simultaneously lift all the axles from the floor bars and in the briefest possible time transfer the load on track 7 to the cooling device B.

65 The cooling device may comprise a water

tank 8, a suitable track 9 above the same, inlet and outlet pipes to circulate the water, and air chambers 10 suspended from the track. These chambers are water tight and they connect with header 11. On the upper side a pair of dampers 12 are horizontally pivoted at each end so as to slide horizontally, as shown in dotted circles at each end of the dampers in Fig. 3. These are operated independently of each other by transverse rock shafts 13 which carry arms 14 that engage the dampers and as the shafts 13 are rocked by hand levers 15 the dampers are opened more or less. It is desirable that they open more rapidly at the center than at the ends of the air chamber 10.

A hood 16 suitably counterweighted drops into tank 8, making an air tight chamber because of the water seal. Air is brought through pipe 17 from a suitable source passing perforated plate 18 into the open space occupied by the steel being treated. Suitable windows and pyrometer openings are provided in the sides of the hood. The hood is raised as shown in dotted lines so as to permit the buggy 5 to pass through under without interference.

When any of the materials require a drawback they may be removed from B 95 by hand or otherwise to the space between it and the furnace A and transferred by traveling crane 19 to the other end of the furnace passing over it and temporarily stored on racks 1 so that the batch being heated in the furnace may be removed by the buggy without interfering with such parts that require re-heating.

It is desirable that axles 20 be suitably spaced on supporting rails 9 of the treatment chamber B in any desired manner, whether placed by hand or mechanism, so as to always lie in the proper position with respect to the air chambers 10.

The heat of the furnace A is very intense 110 and it is ordinarily found difficult to retain permanent metal tracks therein for a transfer buggy to travel on. One way, among many others, to overcome this difficulty is to provide removable rails that may be 115 shoved onto the furnace floor, by means of a hoist 22 operating on a track 21, before the transfer buggy reaches the furnace. These specific details of structure, etc., are embodied in a separate application bearing 120 serial #19,312 filed April 5, 1915.

While in the furnace the materials may rest on suitable bars to permit underneath circulation. They are subjected to a suitable volume of heat, from coal, oil, gas, electricity or any other medium for various lengths of time according to the cubical dimensions of the parts being treated, and in the carrying out of this process to various temperatures according to the carbon con- 125 130

tent of the steel, the range of temperatures being inverse to the variation in carbon. These first steps cause the steel to change into a new structure through a rearrangement of the particles providing the heat is applied gradually. Cold materials should not be placed directly into a hot furnace. When the low critical point of this process determined by previously noted data of a specific carbon is reached the temperature is held uniform for a given time so as to not subject the grains to under stress while the grains are changing positions, etc., thereby effecting a gradual change from coarse particles to fine particles evenly distributed.

The temperature is held for but a fraction of the time required to bring the steel up to this point. Then the heating is continued slowly so as to further refine the grain for a time approximating one-third of the initial heating for smaller pieces and one-half for larger sections until the high critical point is reached, approximately twenty to 25 150 degrees F. higher for the different carbons than the first heat. This difference is a decreasing one as the higher temperatures are reached, being largest for low carbons and practically disappearing when a "saturated" condition is reached at a theoretical content of about 0.89.

As soon as the required highest temperature is reached an allowance of 25 to 50° F. higher being allowed to compensate for the transfer, the steel is quickly removed from the furnace to a suitable treatment apparatus B, which may consist of a hood which incloses the steel in a hermetically sealed compartment, to which air or other 35 cooling agent is supplied in controllable quantity at any desired difference of temperature, and at a pressure which will give a suitable velocity to the cooling agent. This cooling agent may be atmospheric air 40 under pressure, dry steam at about 350° F. or any other gaseous media. Dampers are placed adjacent the steel sections being treated so as to use local treatment if needed.

In ordinary quenching the highest temperature used is below that found desirable when carrying out this process. Should the highly heated steel be suddenly quenched its quality of structure would be lowered, setting up internal strains, breakages, etc. The 50 particles would become fixed, remaining hard and brittle so as to necessitate further treatment to toughen its structure, such re-treatment being however uncertain and not unfrequently hopeless. Such products are a source of great danger when used under critical conditions. The unreliability of quenched steel is aggravated when the sections are of large dimensions because it is 55 impossible to quench such articles without

setting up internal stresses due to a shrinking outside encircling an expanding zone which surrounds a contracting center. The various distances from the center being at different temperatures variable stresses will be set up in objects of circular cross section.

When steel has been mechanically treated under heat it is desirable to allow it to become cold before subjecting it to further heating steps. Whenever the steel after treatment and physical test shows a very high tensile factor, low elastic limit, elongation and reduction of area it may be drawn back by reheating and tempering to approximately 600 to 1200° F. according to the carbon content. The lower carbons are submitted to a temperature approximately three-quarters of that to which the higher carbons are subjected and the period over which these temperatures are applied may range from one to two hours. At any event in order to retain as much of the fine structure secured by the first treatment as possible steel should not again be raised above the low critical point. Should one be uncertain after the first heat as to the tensile quality being too high the steel can be cooled as above and similarly retreated.

The approximate variation of temperatures in relation to the carbon content, etc., may be instanced as follows, for 30 to 65 carbon over a range of about one hundred and fifty degrees Fahrenheit for the first treatment and for the same carbon constituent over a range of approximately 160 degrees F. for the second treatment. The draw back temperatures used in special emergencies for the various carbons mentioned ranges about 360° F. rising with the increase in carbon while the two heat treatment temperatures rise inversely to the increase of carbon. Ordinarily it is found that steels having a carbon content below .40 to .43 require only two consecutive heating stages but those above these percentages may have to be subjected to a draw back because of great brittleness and lack of toughness.

In carrying out the draw back of material having an excessive elastic limit, tensile strength and low elongation and reduction the temperature should be from the lowest point at which steel starts to soften to a degree of temperature below the low critical or change point and kept at that temperature for a time commensurate with the results desired. The temperatures and time allowance though variable to some degree should be checked at frequent intervals by an ordinary pyrometer or more definite comparable results may be secured through the use of a self recording device.

This process is specially applicable to steels of large section in which the elastic limit, tensile strength, elongation and re-

- duction of area must be kept high. A special feature is found in the uniformity of results produced and the absence of failures when products so treated are put to strenuous physical stresses, chemical tests, microscopical determinations, etc. This results in a superior grade of output, not attainable hitherto and notably absent in the usual heat-treatment-quenching processes.
- 10 The ranges of temperature given are only instances of adaptation and not limitations, the important feature being to hold the temperature uniform over the period of time when the particles are rearranging themselves so as not to stress them and give a "set" to their grouping before they are properly refined. To not use a uniform application of heat over this period would seriously modify the quality of steel finally produced.

15 The mean temperature for each carbon content of the first heating stage is approximately the terminal temperature of the second heating corresponding to the same carbon composition. This may be stated in another way. The mean temperature of the second treatment approximates the initial temperatures of the first heat for corresponding percentages of carbon, both 20 stages being consecutive.

25 This process subjects the steel to two ranges of temperature with a rest period between and very rapid controlled cooling, thereby holding the best granular characteristics so as to retain hardness without sacrificing toughness and ductility. The various steps of this process give flexibility yet certainty of control that hitherto has been unattainable and though specially applicable to large sections, such as locomotive axles, etc., wherein the largest safety factors must be embodied, the details are amenable to other purposes. In fact any 30 kind of steel article may be successfully handled in large quantities with uniformity 45 of results.

What I claim is:

1. The process of heat treating steel which consists first of subjecting the material to a continuous rising heat up to about 1370 degrees F. for 30 point carbon and about 1270 degrees F. for 65 point carbon, varying this temperature inversely to the carbon content for intermediate 50 products, arresting the application of heat, and then subjecting the same to a continuous rising temperature above the upper critical point, and finally applying a cooling gaseous medium to reduce the temperature rapidly.

2. The process of heat treatment of steels which consists in heating medium steel (of say 60 to 70 point carbon) for the lower critical point, arresting the application of

heat, again heating to above the upper critical point, and finally quenching in a gaseous cooling medium.

3. The process of heat treating steel after mechanical manipulation which consists in; first, subjecting the same to a continuously rising temperature from a cold state up to about 1390 degrees F. for 30 point carbon and about 1240 degrees F. for steels having approximately twice the carbon content of the former, varying this temperature inversely with the carbon content of intermediate steels; second, arresting the application of heat to maintain a uniform temperature; third, subjecting the material to a continuous rising temperature above the upper critical point, and fourth, rapidly lowering the temperature of the steel by the controlled application of a gaseous medium.

4. The process of treating steels after mechanical manipulation which consists in subjecting a medium steel ranging from about 60 to 70 point carbon to two heating stages separated by an arresting period at about 1340 degrees F. for 50 point carbon during which the temperature is held approximately constant, and finally lowering the temperature rapidly by the application of a gaseous medium, the first heating stage being from a cold state to the arresting point and the second from such point to above the upper critical point.

5. The process of treating medium steels ranging approximately around 30 to 65 point carbon, which consists in gradually raising the temperature from a cold state to about 1370 and 1270 degrees F. respectively, holding the temperature uniform for an appreciable time, again heating to above the upper critical point and finally rapidly reducing the temperature by the application of a gaseous medium without aqueous quenching.

6. The process of heat treatment of steels which consists in slowing and continuously heating the articles from a cold state after hammering for the lower critical point of the process (of say 30 to 70 point carbon), holding the temperature uniform for a time, further continuously heating the articles to above the upper critical point, rapidly cooling the same in a gaseous medium, and finally in case it is necessary to correct for physical test characteristics to subject the material or articles to such draw back temperatures as are needed.

In testimony whereof I affix my signature in presence of two witnesses.

DAVID J. SIMPSON.

Witnesses:

F. W. AMSTUTZ,  
A. L. AMSTUTZ.